# EUROPEAN PATENT SPECIFICATION

(11) **EP 0 837 364 B1**
(45) Date of publication and mention of the grant of the patent: **16.08.2001**
(21) Application number: 97830513.4
(22) Date of filing: 10.10.1997
(51) Int. Cl.: G03C 11/24

(54) **A process for the treatment and recovery of materials from the production and development of photographic and x-ray films**
Verfahren zur Behandlung und Rückgewinnung von Materialien aus der Produktion und Entwicklung photographischer Filme und Röntgenfilme
Procédé de traitement et récupération de matériaux provenant de la production et le développement de films photographiques et radiographiques

(30) Priority: 15.10.1996 IT BO960515
(43) Date of publication of application: 22.04.1998
(73) Proprietor: Serf S.r.l., 40050 Argelato (Bologna) (IT)
(72) Inventor: Miciano, Marino, 40137 Bologna (IT)
(74) Representative: Lanzoni, Luciano

(56) References cited:
- EP-A- 0 239 805
- GB-A- 1 432 000
- US-A- 3 047 435
- US-A- 3 647 422
- US-A- 3 793 168
- US-A- 3 928 253
- US-A- 4 299 676
- US-A- 4 799 954
- US-A- 5 418 115
- DATABASE WPI Section Ch, Week 7907 Derwent Publications Ltd., London, GB; Class E37, AN 79-12657B XP002052387 & JP 54 001 026 A (KONISHIROKU PHOTO IND CO LTD) , 6 January 1979
- DATABASE WPI Section Ch, Week 8747 Derwent Publications Ltd., London, GB; Class M14, AN 87-331438 XP002052388 & JP 62 237 447 A (MITSUBISHI PAPER MILLS LTD) , 17 October 1987
- DATABASE WPI Section Ch, Week 7917 Derwent Publications Ltd., London, GB; Class G06, AN 79-33088B XP002052389 & SU 611 168 A (NONFER METALS HYDRO) , 15 May 1978
- DATABASE WPI Section Ch, Week 9228 Derwent Publications Ltd., London, GB; Class A23, AN 92-232294 XP002052390 & SU 1 681 295 A (KAZAN CHEM PHOTO IND RES DES INST) , 30 September 1991
- COOLEY A C: "SILVER RECOVERY FOR ENVIRONMENTAL COMPLIANCE IN PHOTOGRAPHIC PROCESSING" JOURNAL OF IMAGING SCIENCE AND TECHNOLOGY, vol. 37, no. 4, 1 July 1993, pages 374-379, XP000423013

## Description

The present invention relates to a process for the treatment and recovery of materials from the production and development of photographic and x-ray films. In particular, it relates to a process for the recovery, by means of chemical/physical treatments, of the materials of which photographic films and x-ray plates are made, more precisely the recovery of silver, polyester, which forms the base of the photo-x-ray film, and the animal gelatin which coats one or both surfaces of the aforementioned polyester base.

The present invention, therefore belongs to the sector of industrial chemical processes designed to recover materials which, when recycled, are suitable for further use.

As is known, the recovery of materials from the production and development of photographic and x-ray films currently regards only the metallic part (including the oxidised form) of the said films, that is to say, silver. Obviously, this is due to the intrinsic value of the said metal.

The rest, that is to say, the polyester and gelatin, is currently discarded, this being an undoubted disadvantage from the economic (and environmental) viewpoint, considered that recycled polyester and gelatin have excellent possibilities for re-use. For example, polyester in the textiles sector, and animal gelatin as feed for the bacterial flora in purification plant.

In accordance with conventional techniques, the silver may be recovered using dry or wet systems.

The dry system envisages that the starting material, i.e.: photosensitive plates or films, be subjected to combustion. In this case, the silver evaporates or remains as an unburned base body, which may then be gathered. In contrast, the polyester and gelatin are lost.

As is known, the wet system envisages the use of developing and fixing baths. The fixing bath is used to extract the "superfluous" silver from the fixed silver.

In the document US-4,299,676 is disclosed a process and an apparatus for the recovery of silver from photographic film. The disclosed process comprises the step of (a) shredding or chopping the film material into strips or pieces of predetermined size; (b) bleaching the shredded or chopped film material in a bath of bleach solution to convert the metallic silver present to silver salts that remain on the film material; (c) performing a first stage washing operation in which the bleached film material is washed with first stage wash water; (d) thereafter performing a second stage washing operation in which the bleached film material is washed with a second stage alkaline wash liquid separate and different from and more alkaline than the first stage wash water; (e) fixing the washed film material in at least one bath of fixing solution to remove the silver salts into the fixing solution; (f) collecting and transporting away the film base material from which the silver salts have been removed; and (g) circulating the fixing solution through at least one electrolytic silver recovery unit where the silver is electrolytically deposited on a cathode. The recovered film base material is subjected to a further treatment, such as an enzyme treatment, for the removal of gelatine. However, such enzyme treatment does not recover the gelatine but only its components.

The object of the present invention is, therefore, to recover all of the material, that is to say, the silver, polyester and animal gelatin.

A further object is to effect the said recovery in a relatively simple, low cost manner. These objects, together with others, are all fulfilled by the process for the treatment and recovery of materials from the production and development of photographic and x-ray films, the main characteristics of said process being described in the claims herein. Further characteristics and advantages of the present invention are more clearly illustrated in the following description of the process, by way of example only, and not limited only to the sector protected by the present patent right.

The following is an example of the process.

The material to be treated consists of a base which is a polyester film, coated on one or both surfaces with a gelatin of animal origin, in which metallic silver or silver salt is dispersed.

The material normally arrives in bales of waste or sheets, not yet exposed, or in the form of x-ray plates in envelopes.

The first step, which is manual, consists in undoing the bales and separating the plates from the paper. The film is then shredded in a special machine and reduced to pieces whose size is 0.3 - 3 cm². It is essential that the material be shredded, in order to allow the completion of the chemical reactions which must take place on both surfaces of the film. Larger dimensions would promote adhesion of the surfaces, preventing completion of the reactions and reducing the overall efficiency of the process. In particular, recovery of the silver would be compromised.

The material containing metallic silver is then subjected to a "bleaching" action, that is to say, oxidation of the metallic silver to ionic silver. This action occurs in an aqueous bath, kept at ambient temperature (10 - 25 °C), containing: copper sulphate (to oxidise the silver); hydrogen peroxide (to re-oxidise the copper); sodium chloride (to provide a counter-ion to the silver ion). The reaction occurs at pH 0.5 - 3. Lower pH values could cause the gelatin to be detached; whilst higher pH values would make the bleaching action less effective.

The treatment time varies from 3 to 15 minutes: lower times would be insufficient to complete the reaction; higher times could cause the gelatin to be detached.

The use of copper as an oxidising agent is determined by process economy and final quality of the polyester recovered: other oxidising agents would be more difficult to remove and would, as a result, pollute the final product. The following are the concentrations of the reagents: copper sulphate 5 - 12 %; sodium chloride 5 - 15 %; hydrogen peroxide 0.1 - 1 %.

The material containing bleached silver, that is to say, silver salt, is then treated in a fixing bath containing sodium thiosulphate. During this stage, the silver salt contained in the gelatin, and insoluble in water, is solubilized by the presence of the thiosulphate.

The reaction occurs at pH 4.5 - 5.5; lower pH values would render the thiosulphate unstable, whilst higher values would slow down the extraction-solubilization of the silver salt.

The treatment time is 3 - 15 minutes at a temperature of 5 - 30 °C; the concentration of the sodium thiosulphate may vary from 50 to 200 g/l.

The fixing solution, enriched with silver, is then sent to the electrolytic recuperator; once the silver has been deposited, the bath is put into circulation again.

The material - now consisting of polyester coated with gelatin - is sent to the gelatin removal tank, which consists of a bath containing sodium hydrate 5 - 25 % and is kept at 55 - 80 °C. The gelatin solubilizing process occurs within 5 - 20 minutes.

The polyester is then sent to the washing, rinsing and centrifugation plant.

Afterwards, it is dried until the residual humidity is 0.1 - 3 % and packaged according to market requirements.

The product washing stages may be envisaged upstream of those operating stages which require unpolluted products from the operating stage upstream.

## Claims

1. A process for the treatment and recovery of materials from the production and development of photographic and x-ray films, said materials substantially consisting in a polyester base, coated on one or both surfaces with a gelatin in which metallic silver or silver salt is dispersed, comprising:
- a first stage, involving shredding of the material into pieces with dimensions suitable for promoting the full efficiency of the said process;
- a second stage, involving oxidation of the metallic silver into ionic silver;
- a third stage, for solubilization of the silver salt in water;
- a fourth stage, for recovery of metallic silver by means of electrolysis,
characterised in that the process includes the following further operating stages:
- a fifth stage, for solubilization of the gelatin in an alkaline bath, consisting of a gelatin solubilizing process in a bath containing sodium hydrate 5 - 25 %, kept at a temperature between 55 - 80 °C and for a time within 5 - 20 minutes;
- a sixth stage, for recovery of the gelatin from the alkaline bath;
- a seventh stage, involving washing, rinsing and drying of the polyester from which the silver and gelatin have been removed.

2. The process as described in claim 1, characterised in that it envisages an eighth stage, for drying the polyester until the residual humidity is between 0.1 and 3 %.

3. The process as described in claim 1, characterised in that the dimensions of the said pieces are between 0.3 and 3 cm².

4. The process as described in claim 1, characterised in that the said oxidation of the metallic silver occurs in an aqueous bath containing: copper sulphate, to oxidise the metallic silver; hydrogen peroxide, to re-oxidise the copper, and sodium chloride, to provide a counter-ion to the silver ion; said oxidation occurring in accordance with the preset reaction parameters.

5. The process as described in claim 4, characterised in that the reaction parameters are:
reagent concentrations:
- copper sulphate: 5 - 12 %;
- sodium chloride: 5 - 15 %;
- hydrogen peroxide: 0.1 - 1 %;
- pH values between 0.5 and 3;
- treatment time between 3 and 15 minutes;
- temperature between 5 and 30 °C.

6. The process as described in claim 1, characterised in that the said solubilization of the silver salt occurs in an aqueous bath containing sodium thiosulphate, in accordance with the preset reaction parameters.

7. The process as described in claim 6, characterised in that the reaction parameters are:
- sodium thiosulphate concentration: 50 - 200 g/l;
- pH values between 4.5 and 5.5;
- treatment time between 3 and 15 minutes;
- temperature between 5 and 30 °C.

8. The process as described in claim 1, characterised in that the said solubilization of the gelatin occurs in an aqueous bath containing sodium hydrate, in accordance with the preset reaction parameters.

9. The process as described in claim 1, characterised in that the said washing and rinsing stage occurs in water, and the drying stage is effected by centrifugation.

## Patentansprüche

1. Verfahren zur Behandlung und Rückgewinnung von Materialien aus der Produktion und Entwicklung photographischer Filme und Röntgenfilme, wobei die genannten Materialien im wesentlichen aus einer Polyesterbasis bestehen, beschichtet auf einer oder beiden Oberflächen mit einer Gelatine, in welcher metallenes Silber oder Silbersalz dispergiert ist, enthaltend:
- eine erste Phase des Schnitzelns des Materials zu Stückchen mit solchen Abmessungen, die geeignet sind, die volle Wirksamkeit der genannten Verfahrens zu begünstigen;
- eine zweite Phase der Oxydation des metallenen Silbers zu ionischem Silber;
- eine dritte Phase zum Lösen des Silbersalzes in Wasser;
- eine vierte Phase der Rückgewinnung des metallenen Silbers mit Hilfe der Elektrolyse,
**dadurch gekennzeichnet,** dass das Verfahren die folgenden weiteren Bearbeitungsphasen enthält:
- eine fünfte Phase des Lösens der Gelatine in einem alkalinen Bad, bestehend aus einem Gelatinelösungsverfahren in einem Bad enthaltend Natriumhydrat zu 5 - 25% bei einer Temperatur zwischen 55 - 80°C und für eine Dauer von 5 - 20 Minuten;
- eine sechste Phase der Rückgewinnung der Gelatine aus dem alkalinen Bad;
- eine siebente Phase des Waschens, Spülens und Trocknens des Polyesters, von welchem das Silber und die Gelatine abgezogen wurde.

2. Verfahren nach Patentanspruch 1, **dadurch gekennzeichnet,** dass es eine achte Phase zum Trocknen des Polyesters vorsieht, bis die Restfeuchtigkeit zwischen 0.1 und 3% beträgt.

3. Verfahren nach Patentanspruch 1, **dadurch gekennzeichnet,** dass die Abmessungen der genannten Stückchen zwischen 0.3 und 3 cm² betragen.

4. Verfahren nach Patentanspruch 1, **dadurch gekennzeichnet,** dass die genannte Oxydation des metallenen Silbers in einem wässrigen Bad erfolgt, das wie folgt enthält: Kupfervitriol zum Oxydieren des metallenen Silbers; Perhydrol zum Reoxydieren des Kupfers und Chlornatrium zum Erzeugen eines Gegenions zu dem Silberion; wobei die genannte Oxydation in Übereinstimmung mit den eingestellten Reaktionsparametern erfolgt.

5. Verfahren nach Patentanspruch 4, **dadurch gekennzeichnet,** dass die Reaktionsparameter folgende sind:
Konzentrationen der Reaktionsmittel:
- Kupfervitriol 5 - 12%;
- Chlornatrium 5 - 15%;
- Perhydrol 0.1 - 1%;
- pH-Werte zwischen 0.5 und 3;
- Behandlungsdauer zwischen 3 und 15 Minuten;
- Temperatur zwischen 5 und 30°C.

6. Verfahren nach Patentanspruch 1, **dadurch gekennzeichnet,** dass die genannte Lösung des Silbersalzes in einem wässrigen Bad erfolgt, welches Natriumthiosulfat enthält, immer in Übereinstimmung mit den eingestellten Reaktionsparametern.

7. Verfahren nach Patentanspruch 6, **dadurch gekennzeichnet,** dass die Reaktionsparameter folgende sind:
- Konzentration des Natriumthiosulfats 50 - 200 g/l;
- pH-Werte zwischen 4.5 und 5.5;
- Behandlungsdauer zwischen 3 und 15 Minuten;
- Temperatur zwischen 5 und 30°C.

8. Verfahren nach Patentanspruch 1, **dadurch gekennzeichnet,** dass die genannte Lösung der Gelatine in einem wässrigen Bad erfolgt, enthaltend Natriumhydrat in Übereinstimmung mit den eingestellten Reaktionsparametern.

9. Verfahren nach Patentanspruch 1, **dadurch gekennzeichnet,** dass die genannte Wasch- und Spülphase in Wasser erfolgt und die Trockenphase durch Schleudern ausgeführt wird.

## Revendications

1. Un procédé de traitement et récupération de matériaux provenant de la production et le développement de films photographiques et radiographiques, lesdits matériaux consistant essentiellement en une base de polyester recouverte, sur une ou les deux surfaces, d'une gélatine dans laquelle de l'argent métallique ou du sel d'argent est dispersé, ledit procédé comprenant :
- une première phase de broyage du matériau pour le réduire en morceaux de dimensions adéquates pour favoriser la pleine efficacité du procédé ;
- une deuxième phase d'oxydation de l'argent métallique en argent ionique ;
- une troisième phase de solubilisation du sel d'argent dans de l'eau ;
- une quatrième phase de récupération d'argent métallique par électrolyse,
ledit procédé étant caractérisé en ce qu'il comprend également les phases suivantes :
- une cinquième phase de solubilisation de la gélatine dans un bain alcalin, consistant en un procédé de solubilisation de la gélatine dans un bain contenant de 5 à 25 % d'hydrate de sodium, maintenu à une température de 55 à 80 °C pendant une période de temps de 5 à 20 minutes ;
- une sixième phase de récupération de la gélatine du bain alcalin ;
- une septième phase de lavage, rinçage et séchage du polyester privé de l'argent et de la gélatine.

2. Le procédé selon la revendication 1, caractérisé en ce qu'il prévoit une huitième phase consistant à sécher le polyester jusqu'à ce que l'humidité résiduelle soit comprise entre 0,1 et 3 %.

3. Le procédé selon la revendication 1, caractérisé en ce que les dimensions des morceaux susmentionnés sont comprises entre 0,3 et 3 cm².

4. Le procédé selon la revendication 1, caractérisé en ce que ladite oxydation de l'argent métallique a lieu dans un bain aqueux contenant : du sulfate de cuivre pour l'oxydation de l'argent métallique ; du peroxyde d'hydrogène pour la réoxydation du cuivre, et du chlorure de sodium pour fournir un contre-ion au ion argent ; ladite oxydation ayant lieu selon les paramètres de réaction préétablis.

5. Le procédé selon la revendication 4, caractérisé en ce que lesdits paramètres de réaction sont :
concentration des réactifs :
- sulfate de cuivre : 5 - 12 %
- chlorure de sodium : 5 - 15 %
- peroxyde d'hydrogène : 0,1 - 1 %
- valeurs de pH comprises entre 0,5 et 3 ;
- durée du traitement comprise entre 3 et 15 minutes ;
- température comprise entre 5 et 30 °C.

6. Le procédé selon la revendication 1, caractérisé en ce que ladite solubilisation du sel d'argent a lieu dans un bain aqueux contenant du thiosulfate de sodium, selon les paramètres de réaction préétablis.

7. Le procédé selon la revendication 6, caractérisé en ce que lesdits paramètres de réaction sont :
- concentration du thiosulfate de sodium : 50 - 200 g/l ;
- valeurs de pH comprises entre 4,5 et 5,5 ;
- durée du traitement comprise entre 3 et 15 minutes ;
- température comprise entre 5 et 30 °C.

8. Le procédé selon la revendication 1, caractérisé en ce que ladite solubilisation de la gélatine a lieu dans un bain aqueux contenant de l'hydrate de sodium, selon les paramètres de réaction préétablis.

9. Le procédé selon la revendication 1, caractérisé en ce que ladite phase de lavage et de rinçage a lieu dans de l'eau, et ladite phase de séchage est effectuée par centrifugation.
